

## UNITED STATES PATENT OFFICE.

TAKEO MIYAGUCHI, OF SENDAGAYAMACHI, TOYOTAMAGORI, TOKYOFU, JAPAN.

## METHOD OF CEMENTATION OF BORON INTO THE SURFACE OF IRON OR STEEL.

No Drawing.

Application filed October 19, 1921. Serial No. 508,817.

*To all whom it may concern:*

Be it known that I, TAKEO MIYAGUCHI, subject of the Emperor of Japan, and resident of Sendagayamachi, Toyotamagori, Tokyo, Japan, have invented certain new and useful Improved Methods of Cementation of Boron into the Surface of Iron or Steel, of which the following is a specification.

- 10 My invention relates to improved method of cementation of boron into any desired surface of iron or steel and has for its object the obtaining of tough and hard surface of the metal which is to be utilized in making 15 articles of excellent quality such as bolt heads, knife blades, razor blades, chisels or the like. The further object of the invention is to minimize the wear and tear of the friction surface of shafts, gear wheels, ball 20 bearings or the like.

This invention is an improvement on the method of my copending application Serial No. 508,819 and is also an improvement on the British Patent No. 19461, A. D. 1912. I 25 made exhaustive tests with a view to arriving at an effective and simple method of cementation of boron into the surface of iron or steel.

I have attempted to obtain desired cementation of boron as described in the above British patent by the employment of carbonizing substance such as carbon powder and boron oxide or ferro-boron in an ordinary atmosphere, but I have failed in this 35 way and at last I have succeeded by carrying out the treatment within reducing atmosphere.

In my invention, first, clean the desired surface of iron or steel, then cover the portion where the boron is to be cemented with a mixture of carbon powder and boron oxide, or of carbon powder and boron compound such as borax. The remaining portion is to be shielded with clay or the like in 45 order to prevent the action of boron. Then heat the iron or steel in a furnace up to about 800° or 900° C. in a reducing atmosphere such as provided by gases containing a sufficient quantity of carbon monoxide. 50 The boron in the boron oxide or boron compound becomes reduced by carbon powder with the aid of the reducing atmosphere and the reduced boron penetrates into the surface of the iron or steel to a certain depth.

According to my tests, the cementation of 55 boron and chromium into the surface of iron or steel by diffusion as described in the above British patent was shown as a mere trace and can not afford any beneficial effect to be adapted for commercial use. 60

On the other hand, in my process such cementation of boron into the surface of iron or steel can be secured so as to meet commercial requirements, so that the product thus obtained possesses appreciable 65 characteristics of boron cementation. But the cementation is not so deep as in my copending application although it gives decidedly distinct structure of boron in the 70 surface by microscopic inspection.

This method can be accomplished likewise on the surface of special metals such as metals containing chromium, silicon, nickel, manganese, tungsten, molybdenum or the 75 like.

## What I claim:—

1. A method of cementation of boron into the surface of iron or steel comprising covering the desired surface of the iron or steel with a mixture of carbon powder and boron 80 oxide or compound, and heating it at from 800° C. to 900° C. in a reducing atmosphere.

2. A method of cementation of boron into the surface of iron or steel comprising covering the desired surface of the iron or steel 85 with ferro boron, and heating it at from 800° C. to 900° C. in a reducing atmosphere.

3. A method of cementation of boron into the surface of ferrous alloys comprising, covering the surface of the alloy to be 90 treated with a mixture of carbon powder and boron oxide or compound, and heating it at from 800° C. to 900° C. in a reducing atmosphere.

4. A method of cementation of boron into 95 the surface of ferrous alloys comprising, covering the surface of the alloy to be treated with ferro-boron, and heating it at from 800° C. to 900° C. in a reducing atmosphere.

Signed at the embassy of the United States of America in the Empire of Japan this 26th day of September, A. D. 1921, in presence of two witnesses.

TAKEO MIYAGUCHI.

## Witnesses:

EUGENE W. DOOMENE,  
INGORO WATANABO.